

## UNITED STATES PATENT OFFICE

2,676,149

## STABILIZED GREASE COMPOSITION CONTAINING A STEROL AND A SELENIUM COMPOUND

Harold A. Woods and John A. Edgar, Martinez, Calif., assignors to Shell Development Company, Emeryville, Calif., a corporation of Delaware

No Drawing. Application December 29, 1951,  
Serial No. 264,234

10 Claims. (Cl. 252—42.1)

1

The present invention relates to improvements in grease compositions and more particularly in grease compositions containing a special combination of additive compounds.

Greases comprise a lubricating base gelled to a grease consistency with a gelling agent which may be either an organic material, such as a soap, or an inorganic substance, such as an onium clay, or a colloidal amorphous inorganic oxide or hydroxide, and the like. The presence of the gelling agent complicates research in the determination of the causes of lubrication failure relative to the effect of oxidative breakdown and mechanical influences. Greases have been prepared containing selenium compounds as oxidation inhibitors. However, as the data given hereinafter indicate, the presence of these selenium compounds does not effect satisfactory stabilization of the present compositions.

While many additives are useful at ordinary operation temperatures, certain greases must be stabilized against deterioration and breakdown at temperatures approaching 400–500° F. This is due to the development of machinery containing bearings subject to high temperatures such as in turbo jet engines and in turboprop motors. High temperature greases may be prepared by the gelling of high boiling lubricants with especially favored materials such as the sodium soaps of high molecular weight acids, particularly those having at least 20 carbon atoms. These include the sodium soaps of beeswax acids and of degras as well as inorganic colloids. Certain materials promote the mechanical stability of such greases at high temperatures such as the salts of aromatic acids of which sodium benzoate is a typical example. In spite of the improved performance of such greases at elevated temperatures over ordinary grease compositions, they have not heretofore had satisfactory life as evidenced by the relatively short bearing tests.

It is an object of the present invention to provide improved lubricating greases. It is another object of the present invention to provide greases exhibiting substantially extended bearing life. It is a particular object of this invention to provide greases useful for high temperature operation and which are not subject to mechanical breakdown over extended periods. Other objects will become apparent during the following discussion.

Now in accordance with the present invention it has been found that greases may be stabilized to an unexpected extent by the synergistic cooperation of minor amounts of polycyclic alco-

2

hols and of aliphatic selenium or tellurium compounds as defined hereinafter.

A specific improvement according to the present invention comprises the discovery that high temperature greases comprising a mixture of aliphatic diesters and high boiling petroleum lubricants gelled with sodium soaps of aliphatic acids having at least 20 carbon atoms and containing metallic salts of aromatic acids respond particularly well to the presence of between about 0.25% and about 5% each of wool grease alcohols and dilauryl selenide.

## POLYCYCLIC ALCOHOLS

15 The polycyclic alcohols useful for promoting the stability of the present greases are typified by the sterols. Preferably they are obtained from natural sources and therefore constitute mixtures of alcohols but synthetic materials may be employed if necessary. The following species are typical of the materials which may be employed although natural sources, such as wool fat, are preferred.

|    |                        |                   |
|----|------------------------|-------------------|
| 25 | Allocholesterol        | Alpha-spinasterol |
|    | Ostreasterol           | Fucasterol        |
|    | Lanosterol             | Stigmasterol      |
|    | Lanyl alcohol          | Beta-sitosterol   |
|    | Lano-octadecyl alcohol | Ergosterol        |
|    | Cholesterol            | Ergostanol        |
| 30 | 7-dehydrocholesterol   | Cholestanol       |

While amounts of polycyclic alcohols may vary widely with the specific composition contemplated, they will generally be less than about 5% by weight of the total composition but an effective proportion usually greater than about 0.25%. Optimum results are obtained when the alcohols are present in amounts between about 1% and about 4% by weight of the grease.

## 40 SELENIUM AND TELLURIUM COMPOUNDS

The selenium and tellurium compounds added for their synergistic stabilizing effect have the general configuration:

45  $R-(X)_n-R_1$

wherein R is an aliphatic radical,  $R_1$  is a substituent of the group consisting of hydrogen atoms and aliphatic radicals, X is an element of the group consisting of selenium and tellurium and  $n$  has a value of 1 or 2, said compound containing at least 8 carbon atoms per molecule. Preferably the constituents R and  $R_1$  are aliphatic hydrocarbon radicals and the element X is selenium. The three principal groups of com-



be readily and economically prepared by the following series of reactions:

- (a)  $\text{MCN} + \text{Se} \rightarrow \text{MSeCN}$
- (b)  $\text{RX} + \text{MSeCN} \rightarrow \text{RSeCN} + \text{MX}$
- (c)  $2\text{RSeCN} \rightarrow \text{R}-\text{Se}_2-\text{R} + (\text{CN})_2$

In the above equations, M represents an alkali metal, preferably potassium; R represents an aliphatic group; and X represents a replaceable negative atom or radical, preferably chlorine. In carrying out this process, reaction (a) may be carried out in aqueous solution, reaction (b) may be carried out in ethyl alcohol, and reaction (c) is carried out by reacting the alkyl selenocyanate with caustic alkali in aqueous alcohol. This method does not yield as desirable a product, from the standpoint of lubricant additives, with chlorinated wax as it yields with some of the lower, purer alkyl chlorides, such as lauryl chloride and cetyl chloride.

(4) Selenium is dissolved in strong aqueous or alcoholic caustic soda or caustic potash solution to yield a mixture (in solution) of alkali metal selenides, polyselenides and selenites, possibly also other selenium compounds. It has been found that when this mixture is heated with a halogenated hydrocarbon or mixture of hydrocarbons, such as lauryl chloride or chlorinated wax, the product, comprising a complex mixture of selenides and probably including mono- and diselenides, perhaps also higher polyselenides, is an excellent lubricant additive.

In addition to the mono- and diselenides and their tellurium analogs, seleno- or telluromercaptans are also effective. These selenium compounds are the aliphatic selenomercaptans. Tellurium may be substituted for selenium, although the selenium compounds are preferred. These compounds may be represented by the formula:



wherein  $\text{R}_1$ ,  $\text{R}_2$  and  $\text{R}_3$  are hydrogen or organic radicals (any two of which may be joined to form a single, bivalent radical), C is an aliphatic carbon atom (i. e., a carbon atom other than a carbon atom forming part of a benzenoid ring), and X is selenium or tellurium.

The preferred compounds of the invention are those containing 8 to 30 carbon atoms, most advantageous 10 to 30 carbon atoms in the molecule. As stated, the selenium compounds are preferred to the tellurium compounds.

Examples of selenium and tellurium compounds of the invention are 2-ethylhexyl, decyl, lauryl, cetyl, octadecyl, and "paraffin" selenomercaptans and 2-ethylhexyl, lauryl and octadecyl telluromercaptans. Other radicals (e. g., other alkyl radicals such as undecyl and tetradecyl, aralkyl radicals such as cetylbenzyl and cycloaliphatic radicals such as ethylcyclohexyl and butyl cyclohexyl), may be used in place of the above mentioned radicals, and the organic radical attached to selenium may contain an unsaturated group or may be substituted by a non-hydrocarbon substituent such as chlorine, hydroxyl, alkoxy, amino, etc.

By "paraffin" as used herein to designate an organic radical is meant a radical derived from paraffin wax; e. g., paraffin selenomercaptan is a selenomercaptan (actually, a mixing of selenomercaptan), such as can be prepared by using

chlorinated paraffin wax as the organic chloride, R.Cl, in Equation 2 below.

By "aliphatic" as used herein without qualification to designate an organic radical attached to selenium or tellurium, is meant an organic radical whose attachment to selenium or tellurium is through a non-benzenoid carbon atom; e. g., octadecyl, benzyl and cyclohexyl selenomercaptans are all "aliphatic" selenomercaptans as "aliphatic" is herein defined.

The selenomercaptans can be prepared by the following series of reactions:

- (1)  $\text{Na}_2\text{Se} + \text{Se} \rightarrow \text{Na}_2\text{Se}_2$
- (2)  $\text{Na}_2\text{Se}_2 + 2\text{R.Cl} \rightarrow \text{R.SeSe.R} + 2\text{NaCl}$
- (3)  $\text{R.SeSe.R} + 2\text{H} \rightarrow 2\text{R.SeH}$

Sodium diselenide is prepared by reaction 1 and is reacted with an aliphatic chloride (RCl) in accordance with reaction (2) to yield an aliphatic diselenide (R.SeSe.R). The aliphatic diselenide is reduced in accordance with reaction 3 to yield an aliphatic selenomercaptan.

In reactions 1, 2 and 3, potassium or other metal may be substituted for sodium, tellurium may be used instead of selenium and bromine or other replaceable element or radical may be substituted for chlorine. The group R is an aliphatic group. If a mixed diselenide is available, e. g., octyl cetyl diselenide



it may be substituted for the symmetrical diselenide of reaction 3, yielding a mixture of selenomercaptans (e. g., octyl and cetyl selenomercaptans).

#### LUBRICATING BASE

The present invention contemplates the stabilization of greases generally, regardless of their specific lubricating base. As the data given hereinafter show, certain bases respond to the synergistic additives to a greater extent than others but a beneficial effect has been found in a number of different media. While the stabilization of greases in general is therefore considered the following types of lubricating bases have been found to be particularly responsive.

Petroleum lubricants are valued not only because of their lubricating property but because of economic considerations as well. Moreover they are available in a wide variety of boiling ranges. Since the present invention especially contemplates the production of high temperature greases, it is particularly desirable when petroleum lubricants are present that they have relatively high boiling points and viscosities. It has been found that an especially effective type of lubricating oil comprises one having viscosity of between about 1250 and 11,000 SUS at 100° F. In order to promote the stability of such mineral oils it is preferred that they contain less than about 15% by weight of aromatic hydrocarbons.

While the present invention is not to be confined to the use of a mineral oil derived from any particular source or by any particular refining process, the usual source of suitable mineral oils comprises the fraction thereof generally termed "bright stocks," and particularly bright stocks having a viscosity index of at least 60. The term "bright stock" is one which is well recognized in the art of refining mineral oils. To obtain the desired fraction, crude oils are usually subjected to distillation under ordinary pressures in order to obtain a "long residue" comprising the fraction which does not distill under these conditions without substantial decomposition. The long

residue is then subjected to steam distillation, usually under a vacuum. Under these conditions, gas oil and waxy lubricant fractions distill over, leaving what is normally termed a "short residue" or a "steam refined stock," also known as "cylinder stock." The steam refined stock is then deasphalted (if an asphaltic crude is employed) and subjected to dewaxing operations to remove microcrystalline or macrocrystalline waxes. Following this, the raffinate is treated with a solvent for the purpose of reducing or removing the aromatic fractions. Clay contact treatment or percolation may be employed to clean up the oil following any one or all of these separate operations. The raffinate which remains after reasphalting, dewaxing, extraction, and clay treatment is generally called "bright stock."

The bright stocks suitable for use in the present compositions should have the following ranges of properties:

Table I

## PROPERTIES OF BRIGHT STOCKS

Visc., SUS, 100° F., >1250, usually 1250-11,000, preferably 1500-3500  
 Visc., SUS, 210° F., >75, usually 125-325, preferably 150-250  
 V. I., >+60, preferably +85-110  
 Aniline point, °C., >100, preferably >115  
 Flash, °F., >475, preferably >500  
 Fire, °F., >550, preferably 600  
 Pour point, °F., maximum 25, preferably lower than 15  
 Per cent aromatics, <15, preferably <10 optimum <5  
 Per cent naphthenes, <35  
 Per cent paraffines, at least 60

The tables which follow give the properties of typical bright stocks which are useful in the compositions of this invention.

Table II  
EXAMPLES OF TYPICAL BRIGHT STOCKS

|                             | Viscosity SUS at °F. |         | Ring Analysis <sup>1</sup> |             |            |            | Ratio P/N | Av. Mol. Wt. | Av. Rings per Mol. |
|-----------------------------|----------------------|---------|----------------------------|-------------|------------|------------|-----------|--------------|--------------------|
|                             | 100° F.              | 210° F. | VI                         | Ar, percent | N, percent | P, percent |           |              |                    |
| Mid-Continent Bright Stock: |                      |         |                            |             |            |            |           |              |                    |
| Conventional Extraction     | 3,650                | 164     | 77                         | 13          | 17         | 70         | 4.1       | 685          | 3.7                |
| Mild Extraction             | 2,569                | 141     | 85                         | 9           | 19         | 72         | 3.8       | 685          | 3.4                |
| Heavy Extraction            | 2,049                | 131     | 93                         | 3           | 21         | 76         | 3.62      | 675          | 2.9                |
| Pennsylvania Bright Stock   | 2,109                | 144     | 102                        | 5           | 16         | 79         | 4.95      | 730          | 3.0                |
| Coastal Bright Stock        | 1,251                | 85      | 63                         | 4           | 35         | 61         | 1.74      | 515          | 3.4                |

<sup>1</sup> Ar=aromatics, N=naphthenes, P=paraffins.

Table III  
SPECIFICATIONS FOR TYPICAL MID-CONTINENT BRIGHT STOCKS

|                     | Unfiltered | Filtered |
|---------------------|------------|----------|
| Gravity, °API, min. | 24.5       | 25.5     |
| Color, NPA          | Dark Green | 6.7      |
| Pour Pt. °F., max.  | 10         | 10       |
| Flash °F., min.     | 580        | 545      |
| Fire °F., min.      | 655        | 610      |
| SUS °F., 210        | 200-215    | 150-160  |
| VI, min.            | 90         | 90       |

It will be understood from the above analyses that the source of treatment of a particular mineral oil is not as important for the present purpose as the final properties of the mineral oil constituent to be used in these compositions. For example, it is possible to vary the extent of solvent extraction dependent upon the original

aromatic content and the requirements of the specific use of the final product, as well as upon the necessity or desirability of deasphalting, clay treating, acid treating, and the like. Hence, it will be recognized that the present invention is predicated upon the use of a mineral oil fraction having the above defined ranges of properties and not upon the source of treatment of such oil.

The most important inherent properties of a mineral oil suitable for the present use comprise the volatility, oxidation stability, aromatic content and viscosity characteristics. The aromatic content has a large influence upon the sensitivity of the oil to thermal changes and the viscosity of the oils defines their suitability for their present purpose. Hence, the best definition with respect to essential characteristics of mineral oil suitable for the present compositions comprising those having an aromatic hydrocarbon content less than about 15% by weight and having a viscosity of between about 1250 and about 11,000 SUS at 100° F. Having defined these particular properties, the other properties such as flash, fire, aniline point, and viscosity index usually are largely dependent upon them.

While mineral oils, such as those described above, may be used as the sole lubricating base, it has been found that certain advantages are gained by combining it with synthetic lubricants such as aliphatic diesters or polyorganosiloxanes.

The term "polyorganosiloxane" as used herein embraces those organic polymers having the unit structure:



wherein the units are attached through the silicon and oxygen atoms and wherein R and R'

represent alkyl, aryl, alkaryl, aralkyl, and cycloalkyl groups. The method of producing these polymers is well known, and may involve the reaction of a silicon halide with a Grignard reagent to form the corresponding organo silicon halide, followed by hydrolysis of the organo silicon halide to form a silicol, and then condensation of the silicol in the presence of air or oxygen, with the aid of a catalyst or heat to form the polyorganosiloxane or silicone polymer (Kipping, Proc. Chem. Soc. 20, 15-16 (1904)). Depending upon the extent of condensation or polymerization, the resulting products vary from relatively light liquids to solid resins and are reported to be both chain-like (U. S. Patent No. 2,352,974—Rochow) and cyclic (U. S. Patent No. 2,371,050—Hyde) in structure. For purposes of the present invention, only those polymers which are high boiling liquids within the lubricating oil

viscosity range are suitable, these generally possessing a viscosity of 100° F. within the range of about 10-600 centistokes. These polyorganosiloxane liquids within this viscosity range are generally colorless, odorless and relatively inert, have very low volatility, such that vapor pressure within the lubricating temperature range is substantially negligible, and high viscosity index which means that they undergo relatively little change in viscosity for a given change in temperature.

While any of the various types of silicone polymers within the foregoing definition are contemplated for purposes of the present invention, the preferred polymers, from the standpoint of cost, are those which have achieved the greatest commercial production, namely, the dimethyl silicone polymers, the diethyl silicone polymers, and the ethylphenyl or methylphenyl silicone polymers. However, it is contemplated that the silicone polymers produced from higher molecular weight alkyl groups, such as butyl, amyl and above, when economically available, will constitute valuable lubricant bases for purposes of the present invention. In general, these silicone polymers are adapted to specialized lubrication outside the conventional lubricating temperature ranges, such as ultra low temperature operation found in refrigerator systems and arctic service, or to general purpose lubrication over a wide lubricating temperature range which was previously unattainable through the use of a single mineral lubricating oil because of the latter's high viscosity change over such a wide temperature range. In addition, these silicone materials are more resistant at high temperatures where hydrocarbons, esters of carbon chain compounds, and similar synthetic lubricant bases of essentially organic structure are subject to carbonization such that they eventually become dry and hard.

Aliphatic diesters are suitable lubricating components in the present greases. The aliphatic diesters to be used in place of, or in combination with, other lubricating bases described herein are preferably those formed by esterification of an aliphatic dicarboxylic acid and of an aliphatic monohydric alcohol having between 2 and 20 carbon atoms. While these are generally of the type described in U. S. Patent 2,481,372, the preferred classification includes especially the aliphatic esters of dicarboxyalkanes wherein said alkane contains between about 4 and 20 carbon atoms and preferably between 4 and 12 carbon atoms. Typical species meeting these requirements include especially the branched chain alkyl diesters such as di(1-ethylpropyl)oxalate, di(2-ethylhexyl)oxalate, di(2-ethylhexyl)sebacate, di(2-ethylhexyl)succinate, di(dodecyl)sebacate and other esters of aliphatic monohydric alcohols with acids such as malonic, succinic, glutaric, adipic, and sebaceous acid.

When mineral lubricating oils are combined in the present compositions with synthetic materials such as the aliphatic diesters or the polyorganosiloxanes, the proportion may vary within wide limits. It has been found, however, that certain proportions exhibit optimum response to the particular combination of additives claimed and described herein. It is preferred, therefore, that the proportion of mineral oil to synthetic lubricant be within the limits from about 3:1 to about 1:3. More particularly the ratio should be confined to proportions between about 2:1 and 1:2 if the best results are desired.

In addition to the above types of materials, other lubricants may be used such as organic phosphates and silicates including tricresyl phosphate, trioctyl phosphate and tetraoctyl silicate.

- 5 5 Certain other phosphorous additives are indicated such as the phosphonates and phosphinates. Typical species of these include: Bis(3,5,5-trimethylhexyl); 2,4,4-trimethyl pentane phosphonate; tris(3,5,5-trimethylhexyl)phosphate; 10 2-ethylhexyl bis(4-tetradecyl) phosphinate as well as diphosphorus compounds of which the following are typical: Bis-1,4-(secondary amyl pentane phosphino)butane; 1,6-hexane diol di(bis-butyl phosphate); 1,5-pentane diol di(butyl butane phosphate); bis-1,3-diisobutyl phosphono)pentane.

It will be understood that the lubricant or mixture of lubricants employed in these compositions constitute the major ingredient thereof. The precise amount which is present is not a critical feature of this invention since the stability of the compositions depends upon the presence of the two synergizing additives rather than upon the exact proportion of the lubricating ingredients.

25

#### GELLING AGENTS

As stated hereinbefore, the grease may be gelled to an appropriate consistency by the presence of organic or inorganic gelling agents. Usually

- 30 30 these will comprise soaps of high molecular weight acids, preferably having at least 20 carbon atoms and being of an aliphatic character. Generally they are saturated or unsaturated aliphatic monocarboxylic acids preferably derived from natural sources such as from beeswax or debras. The following list of acids is typical of those particularly effective for use in greases to be inserted in machinery operated at relatively high temperatures:

- 40 40 Phthioic acid  
Tetracosanoic acids (e.g., selacholeic acid)  
Docosanoic acids (e.g., ereic acid)  
Eicosanoic acids (e.g., gadoleic acid)  
Arachidonic acid  
45 45 Clupanodonic acid  
Lignoceric acid  
Selacholeic acid  
Cetoleic acid  
Melissic acid  
50 50 Montanic acid  
Cerotic acid  
Behenic acid  
n-Octatriacontanoic acid

- 55 55 While acids having more than about 20 carbon atoms are preferred for the special purpose of preparing high temperature greases other high temperature greases may be prepared by the use of inorganic gelling agents and particularly from amorphous colloidal gelling materials such as silica, magnesia, lime and mixtures thereof. The so-called "microgels" having surface areas of at least about 100 square meters per gram may be prepared according to known methods and

- 60 60 may comprise mixtures of inorganic gelling agents with organic materials such as soaps or amines. When high temperature requirements are not paramount, soaps of lower molecular weights may be used such as the sodium, potassium or lithium soaps of fatty or hydroxy fatty acids including lithium 12-hydroxy stearate, sodium stearate, calcium oleate and the like. Other metallic soaps include those of amphoteric metals or heavy metals such as copper, aluminum, magnesium, calcium, iron and similar materials

75 75 and 1:2 if the best results are desired.

known for their soap-forming properties. Preferably the soaps or other gelling agents are present in amounts between about 2% and 25% by weight of the total grease composition. Usually they are present in amounts between about 5% and 15%.

#### OTHER INGREDIENTS

In addition to the essential components of the greases, as given in detail hereinbefore, other optional ingredients may be present. One of the most important of these comprises the salts of organic carboxylic acids containing an aromatic ring. The presence of such salts has been found to unaccountably increase the dropping point of greases and, hence, to promote optimum properties in greases for use at high temperatures. The alkali metal salts are especially preferred such as the sodium potassium or lithium salts of benzoic acid or alkyl benzoic acids including phenyl acetic or toluic acids. Similar results are obtained by the use of metallic salts of hydrocinnamic acid, as well as from the sodium salt of aromatic poly basic acid such as sodium phthalate. Such salts are preferably present in amounts between about 0.2% and 5% based on the weight of the total grease.

In order to promote the maximum stability against oxidation, aromatic amines are also employed such as phenyl - alpha - naphthylamine, phenyl-beta-naphthylamine and phenylene diamine. Useful additives for the improvement in corrosion characteristics include especially the reaction products of a phosphorous sulfide and a terpene such as the reaction product of phosphorus pentasulfide and turpentine. Moreover, the metallic salts of substituted thiocarbamic acids also may be included such as the zinc, calcium or magnesium salts of alkyl thiocarbamic acids including zinc dibutyl dithiocarbamate, calcium ethylhexyl dithiocarbamate, magnesium dioctyl dithiocarbamate and the like. These additives should be employed in minor amounts, preferably less than 5% of the total amount of the grease, but as least in amounts of about 0.25%.

In addition to the above materials the compositions may contain thickeners and viscosity index improvers such as the polymeric acids of the acrylic acid series or polymeric olefins having molecular weights greater than about 1,000. Typical species of these substances include the lower alkyl esters (ethyl through octyl) of polymethacrylic acids having molecular weights between about 5,000 and 25,000 and polybutene or polyisobutene having molecular weights of between about 8,000 and 20,000.

The following examples illustrate the advantages to be gained by the use of compositions according to the present invention.

The greases to be described were prepared by the following process which is described as merely typical of a number of means for assembling the constituents into a grease composition. Part of the lubricating base was heated to a temperature of about 195° F. at which temperature beeswax was added and stirred until melted in the lubricant. While heating to a temperature of about 230° F., concentrated sodium hydroxide solution was added with stirring. Water was eliminated by continued heating up to a temperature of about 300° F. at which point the soap and oil were held for a period of about one hour. The blend was then cooled to a temperature of about 195° F., at which point wool grease alcohols or their equivalent were added together with about 1% by weight of water based on the total

grease. Thereafter the mixture was reheated to a temperature of about 450° F. for a period of about thirty minutes. The temperature was then reduced by the addition of the balance of the oil and, if necessary, by the use of external cooling. At a temperature of approximately 160° F. the remainder of the additives, as specified in the following examples, was added and the greases homogenized to obtain smooth products.

- 5 10 It will be appreciated by experts in the art that the steps involved in the above process may be amended to suit the particular composition being prepared. If the actual steps enumerated are employed the temperatures may be varied approximately 50°, suitable to cause either solution of the desired product in the oil or saponification of the particular acid utilized. Moreover the period of heating or cooling and the period of holding at that particular temperature may be varied without departing from the spirit of the present invention. Table IV, given below, illustrates the effect of preparing greases having both dilauryl selenide and wool grease alcohols upon the operating life of the resulting greases. These 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195

In the above table it will be found that the greatest response was shown by a lubricating base comprised of equal proportions of a petroleum oil bright stock and of an aliphatic diester. When the proportion of bright stock was increased, the test life of the resulting grease was substantially reduced. In the absence of any aliphatic diester, a still further reduction in the life of the grease occurred.

Table VI illustrates the effect of operating the grease at high temperatures when employing lubricating bases composed entirely, or in part, of a polyorganosiloxane, namely, a dimethyl silicone fluid.

Table VI

| Sample | Ratio, Bright Stock-Silicone | Dilauryl Selenide, Percent | Wool Grease Alcohols, Percent | ABEC Test 400° F., 10,000 R.P.M. Hours to Failure |
|--------|------------------------------|----------------------------|-------------------------------|---------------------------------------------------|
| G      | 0:1                          | 1                          | 0                             | 170                                               |
| H      | 0:1                          | 1                          | 3                             | 238                                               |
| I      | 0:1                          | 0                          | 3                             | 20                                                |
| J      | 3:17                         | 1                          | 0                             | 176                                               |
| K      | 3:17                         | 0                          | 3                             | 100                                               |
| L      | 3:17                         | 1                          | 3                             | 27                                                |

While the above examples illustrate the synergistic effect obtained by the presence of the two required additives, the following examples illustrate other embodiments of this invention:

## Example I

|                    |      |
|--------------------|------|
| Lithium stearate   | 18.0 |
| Mineral oil        | 78.0 |
| Dicetyl diselenide | 0.5  |
| Cholestanol        | 3.5  |

## Example II

|                                     |      |
|-------------------------------------|------|
| Lithium 12-hydroxy stearate         | 12.5 |
| Poly(propylene oxide) mol. wt. 1250 | 84.2 |
| Ethyl octadecyl selenide            | 0.8  |
| Cholesterol                         | 2.5  |

## Example III

|                            |      |
|----------------------------|------|
| Barium stearate            | 15.0 |
| Bis(2-ethylhexyl) sebacate | 41.0 |
| Bright stock mineral oil   | 41.0 |
| Octadecyl selenomercaptan  | 1.0  |
| Lanyl alcohol              | 2.0  |

## Example IV

|                             |      |
|-----------------------------|------|
| Sodium soap of degras       | 12.0 |
| Dihexyl benzene phosphonate | 30.0 |
| Mineral oil                 | 51.0 |
| Didecyl selenide            | 1.5  |
| Allocholesterol             | 3.0  |
| Sodium cinnamate            | 2.5  |

## Example V

|                               |       |
|-------------------------------|-------|
| Sodium soaps of beeswax acids | 10.0  |
| Bright stock                  | 33.75 |
| Bis(diisobutyl) sebacate      | 50.0  |
| Wool grease alcohols          | 1.5   |
| Dilauryl selenide             | 0.25  |
| Zinc dibutyl dithiocarbamate  | 1.5   |
| Sodium benzoate               | 3.0   |

## Example VI

|                                                                  |      |
|------------------------------------------------------------------|------|
| Sodium soaps of beeswax acids                                    | 10.0 |
| Bis(didecyl) sebacate                                            | 41.5 |
| Bright stock                                                     | 40.0 |
| Wool grease alcohols                                             | 3.0  |
| Ditetradecyl selenide                                            | 1.0  |
| Sodium benzoate                                                  | 3.0  |
| Zinc dibutyl dithiocarbamate                                     | 0.5  |
| Reaction product of turpentine and P <sub>2</sub> S <sub>5</sub> | 1.0  |

## Example VII

|                                                                  |      |
|------------------------------------------------------------------|------|
| Sodium soaps of beeswax acids                                    | 10.0 |
| Bis(dodecyl) sebacate                                            | 40.5 |
| Bright stock                                                     | 40.0 |
| Wool grease alcohols                                             | 3.0  |
| Didecyl selenide                                                 | 1.0  |
| Sodium benzoate                                                  | 3.0  |
| Zinc dibutyl dithiocarbamate                                     | 0.5  |
| Reaction product of turpentine and P <sub>2</sub> S <sub>5</sub> | 1.0  |
| Phenyl-alpha-naphthylamine                                       | 1.0  |

We claim as our invention:

1. A grease composition comprising a major proportion of a lubricating oil, a grease-forming proportion of a gelling agent, and minor amounts, but sufficient to increase the operating life of said grease, of a sterol and of a compound of the type



20 where R is an aliphatic radical, R<sub>1</sub> is a substituent of the group consisting of hydrogen atoms and aliphatic radicals, X is an element of the group consisting of selenium and tellurium, and n is a full integer less than 3, said compound containing at least 8 carbon atoms per molecule.

25 2. A grease composition comprising a major proportion of a lubricating oil, a grease-forming proportion of a metallic soap, and minor amounts less than about 5%, by weight, each but sufficient to increase the operating life of said grease of a sterol and of a dialkyl monoselenide containing at least 8 carbon atoms per molecule.

30 3. A grease composition comprising a major proportion of a mixture of an aliphatic diester and of a petroleum lubricating oil having a viscosity between about 1250 and 11,000 SUS at 100° F. and containing less than about 15% by weight of aromatic hydrocarbons, between about 2% and 25% by weight of a soap of an aliphatic monocarboxylic acid, and minor amounts less than about 5% by weight each but sufficient to increase the operating life of said grease of a sterol and of a dialkyl monoselenide containing at least 8 carbon atoms per molecule.

35 4. A grease composition comprising a major proportion of a mixture of an aliphatic diester and of a petroleum lubricating oil having a viscosity between about 1250 and 11,000 SUS at 100° F., between about 2 and 25% by weight of a sodium soap of an aliphatic monocarboxylic acid having at least 20 carbon atoms per molecule, and minor amounts less than about 5% by weight each but sufficient to increase the operating life of said grease of a sterol and of a dialkyl monoselenide containing at least 8 carbon atoms per molecule.

40 5. A grease composition comprising a major proportion of a mixture of an aliphatic diester and a petroleum lubricating oil having a viscosity between about 1250 and 11,000 SUS at 100° F., between about 2% and about 25% by weight of a sodium soap of at least 1 aliphatic monocarboxylic acid having at least 20 carbon atoms per molecule and minor amounts less than about 5% by weight each but sufficient to increase the operating life of said grease of a sterol and of a dialkyl monoselenide containing at least 8 carbon atoms per molecule.

45 6. A grease composition comprising a major proportion of a mixture of an aliphatic diester and of a petroleum lubricating oil having a viscosity between about 1500 and 3500 SUS at 100° F. and containing less than about 10% by weight of aromatic hydrocarbons, between about 2% and about 25% by weight of sodium soaps of bees-

wax acids and minor amounts less than about 5% by weight each but sufficient to increase the operating life of said grease of wool grease alcohols and dilauryl selenide.

7. A grease composition comprising a major proportion of a lubricating oil comprising a mixture of an aliphatic diester and a petroleum lubricating oil having a viscosity between about 1500 and about 3500 SUS at 100° F. and containing less than about 10% by weight of aromatic hydrocarbons, between about 2% and about 25% by weight of sodium soaps of beeswax acids and minor amounts less than about 5% by weight each but sufficient to increase the operating life of said grease of cholesterol, dilauryl selenide, and sodium benzoate.

8. A grease composition comprising a major proportion of a lubricating oil, grease-forming proportions of a metallic soap of a higher aliphatic acid and minor amounts less than about 5% each but sufficient to increase the operating life of said grease of a sterol and of a dialkyl diselenide containing at least 8 carbon atoms per molecule.

9. A grease composition comprising a major

proportion of a lubricating oil, grease-forming proportions of a metallic soap of a higher aliphatic acid and minor amounts less than about 5% each but sufficient to increase the operating life of said grease of a sterol and of an alkyl selenomercaptan.

10. A grease composition comprising a major proportion of a mixture of lubricating oils comprising a polyorganosiloxane and a petroleum lubricating oil having a viscosity between about 1250 and 11,000 SUS at 100° F., between about 2% and about 25% by weight of sodium soaps of degras acids and minor amounts less than about 5% by weight each but sufficient to increase the operating life of said grease of octadecyl selenomercaptan, cholesterol and a metallic salt of an aromatic acid.

References Cited in the file of this patent

UNITED STATES PATENTS

| Number    | Name           | Date          |
|-----------|----------------|---------------|
| 2,398,415 | Denison et al. | Apr. 16, 1946 |
| 2,556,289 | Morway         | June 12, 1951 |